



US005634370A

**United States Patent** [19]

Anthony et al.

[11] Patent Number: **5,634,370**[45] Date of Patent: **Jun. 3, 1997**[54] **COMPOSITE DIAMOND WIRE DIE**[75] Inventors: **Thomas R. Anthony**, Schenectady, N.Y.; **Bradley E. Williams**, Worthington, Ohio[73] Assignee: **General Electric Company**, Schenectady, N.Y.[21] Appl. No.: **499,502**[22] Filed: **Jul. 7, 1995**[51] Int. Cl.<sup>6</sup> ..... **B21C 3/00**[52] U.S. Cl. ..... **72/467**[58] Field of Search ..... **72/467; 423/446**[56] **References Cited**

## U.S. PATENT DOCUMENTS

|           |         |                     |         |
|-----------|---------|---------------------|---------|
| 3,433,049 | 3/1969  | Neaser et al.       | 72/467  |
| 3,831,428 | 8/1974  | Wentorf, Jr. et al. | 72/467  |
| 4,016,736 | 4/1977  | Carrison et al.     | 72/41   |
| 4,303,442 | 12/1981 | Hara et al.         | 72/467  |
| 4,392,397 | 7/1983  | Engelfriet et al.   | 72/467  |
| 4,462,242 | 7/1984  | Morgenthaler        | 72/467  |
| 4,872,333 | 10/1989 | Burnand             | 72/467  |
| 5,110,579 | 5/1992  | Anthony et al.      | 423/446 |
| 5,273,731 | 12/1993 | Anthony et al.      | 423/446 |
| 5,310,447 | 5/1994  | Anthony et al.      | 423/446 |
| 5,360,479 | 11/1994 | Banholzer et al.    | 117/84  |
| 5,361,621 | 11/1994 | Anthony et al.      | 72/467  |

|           |         |                |          |
|-----------|---------|----------------|----------|
| 5,363,687 | 11/1994 | Anthony et al. | 72/467   |
| 5,377,522 | 1/1995  | Anthony et al. | 72/467   |
| 5,387,447 | 2/1995  | Slutz et al.   | 428/34.1 |
| 5,511,450 | 4/1996  | Nagao          | 72/467   |

## FOREIGN PATENT DOCUMENTS

|          |        |                    |   |
|----------|--------|--------------------|---|
| 024757   | 3/1981 | European Pat. Off. | . |
| 494799A1 | 1/1992 | European Pat. Off. | . |
| 531085   | 3/1993 | European Pat. Off. | . |

## OTHER PUBLICATIONS

Wilks, John and Eileen Wilks. "Properties and Applications of Diamond". Oxford, U.K. 1991. Chapter 17, Miscellaneous applications. pp. 504-507.

Wilks, John and Eileen Wilks. "Properties and Applications of Diamond". Oxford, U.K. 1991. Chapter 13, Wear and surface characteristics. pp. 337, 342, 343, and 377.

Primary Examiner—David Jones  
Assistant Examiner—John Paradiso  
Attorney, Agent, or Firm—William H. Pittman

[57] **ABSTRACT**

A composite diamond wire die for drawing wire has a single crystal or HTHP diamond substrate and a CVD layer or layers deposited thereon. The wire die bore extends through the diamond substrate, and the substrate is surrounded by the diamond CVD layer.

25 Claims, 2 Drawing Sheets





FIG. 1



FIG. 2



FIG. 3



Fig. 4

## COMPOSITE DIAMOND WIRE DIE

## FIELD OF THE INVENTION

This invention is related generally to diamond dies for wire drawing. More particularly, it is related to a composite diamond die comprising portions made from both CVD and natural or HPHT diamond.

## BACKGROUND OF THE INVENTION

Wires of metals such as tungsten, copper, iron, molybdenum, and stainless steel are produced by drawing the metals through diamond wire dies. Diamond wire dies have been fabricated using single crystal diamonds, however, such dies are difficult to fabricate, tend to chip easily, easily cleave, and often fail catastrophically in use because of the extreme pressures involved during wire drawing.

With reference to single crystal diamond wire dies, it is reported in Properties and Applications of Diamond, Wilks et al, Butterworth-Heinemann Ltd 1991, pages 505-507: "The best choice of [crystallographic] direction is not too obvious because as the wire passes through the die its circumference is abrading the diamond on a whole 360° range of planes, and the rates of wear on these planes will be somewhat different. Hence, the originally circular hole will not only grow larger but will lose its shape. However, <110> directions offer the advantage that the wire is abrading the sides of the hole with {001} and {011} crystallographic orientations in abrasion resistant directions."

Diamond dies which avoid some of the problems attendant with natural diamonds of poorer quality comprise microporous masses compacted from tiny crystals of natural or synthesized diamonds or from crystals of cubic boron nitride. The deficiencies of such polycrystalline hard masses, as indicated in U.S. Pat. No. 4,016,736 to Carrison et al., are due to the presence of micro-voids/pores and soft inclusions. These voids and inclusions can be more than 10 microns in diameter. The improvement of Carrison et al. incorporates an impregnated lubricant in the microporous wire die and a metal cemented carbide jacket to enclose the die.

European Patent Application 0 494 799 A1 describes a polycrystalline CVD diamond layer having a hole formed therethrough and mounted in a support. As set forth in column 2, lines 26-28, "The relatively random distribution of crystal orientations in the CVD diamond ensures more even wear during use of the insert." As set forth in column 3, lines 50-54, "The orientation of the diamond in the polycrystalline CVD diamond layer 10 may be such that most of the crystallites have a (111) crystallographic axis in the plane, i.e. parallel to the surfaces 14, 16, of the layer 10."

Other crystal orientations for CVD films are known. U.S. Pat. No. 5,110,579 to Anthony et al describes a polycrystalline diamond film comprising substantially transparent columns of diamond crystals having a <110> direction perpendicular to the base, as illustrated in FIG. 3 of this patent.

As discussed in, for example, U.S. Pat. Nos. 5,361,621, 5,363,687 and 5,377,522, CVD diamond has been preferred for wire die applications because of its high purity and uniform consistency. Natural diamonds typically are less pure compositionally, and have less morphological consistency. Also, because CVD diamond usually can be produced without attendant voids, it is often more desirable than polycrystalline or single crystal diamond produced by high temperature and high pressure (HPHT) processes. However,

the surfaces of CVD diamonds used for wire dies have been observed in some instances to contain pits or voids after the polishing operations used to form the surfaces of the die, or after wire drawing. These pits or pores may result from the CVD deposition process or from pull-out of fine grains during these operations. Pull-out may result from relatively low grain boundary strength, which may in turn be related to the CVD deposition process. CVD deposited carbon films are known to contain hydrogen that is bonded to the carbon, particularly in the grain boundaries, which in turn results in a reduction in the number of carbon-carbon bonds across the grain boundaries, and hence, a reduction in the grain boundary strength. The degree of pitting observed is greater than that which occurs when natural diamonds that are subject to the same die forming operations.

Pits or pores are of concern, because they are expected to limit the maximum strength of wire dies in which they occur and, therefore, the types of wire that may be formed in them (e.g. relatively ductile alloys such as many copper alloys versus less ductile alloys, such as most tungsten alloys). Pits or voids may also cause defects in the drawn wire, particularly if they occur in the bearing surface of the die, where most of the wire deformation occurs.

Therefore, it is desirable to combine single crystal and CVD diamond to make composite diamond wire dies that take advantage of the properties and characteristics of both.

## SUMMARY OF THE INVENTION

A composite diamond wire die combines the advantages of natural and HPHT diamond with the advantages of CVD diamond. A relatively small piece of natural or HPHT diamond is used as a substrate for a layer or layers of CVD diamond. The CVD diamond is used to add sufficient material to the substrate to permit the fabrication of a diamond wire die.

The present invention may be briefly described as a composite diamond wire die for drawing wire of a predetermined diameter, comprising: a substrate comprising natural or HPHT diamond and having a top surface, a bottom surface and a lateral surface located between the top and bottom surfaces; a layer of CVD diamond deposited on the lateral surface of said substrate (lateral layer); and at least one wire die bore comprising a wire bearing portion of substantially circular cross-section and a bore axis, said wire die bore extending from the top surface to the bottom surface through the substrate and surrounded by the CVD diamond layer, wherein the circular cross-section of the wire bearing portion is determinative of the diameter of a wire drawn through said wire die bore.

In a preferred embodiment, a wire die of the present invention has a wire die bore extending entirely through the die along a bore axis where the substrate has a <110> direction extending substantially parallel to the bore axis.

One object of the present invention is to produce a diamond wire die that is less susceptible to voids or pullout within the wire die bore. Another object of the present invention is to provide a diamond wire die that can draw wire with higher yield strengths than may be drawn with CVD diamond wire dies. A further object is to provide a diamond wire die that is constructed from less costly materials than dies made entirely from single crystal natural diamonds.

## BRIEF DESCRIPTION OF THE DRAWINGS

FIGS. 1 is a cross-sectional illustrations of a composite diamond wire die of the present invention.

FIG. 2 is a top view of one embodiment of the wire die of FIG. 1.

FIG. 3 is a top view of a second embodiment of the wire die of FIG. 1.

FIG. 4 is a cross-sectional illustration of another embodiment of a composite diamond wire die of the present invention.

#### DETAILED DESCRIPTION OF THE INVENTION

FIG. 1-3 are cross-sectional and top view illustrations of several embodiments of a composite diamond wire die 10 of the present invention. Wire die 10 is for drawing wire (not shown) of a predetermined diameter, and comprises: substrate 12 comprising natural or HPHT diamond and having a top surface 14, bottom surface 16 and lateral surface 18; a layer 20 of diamond deposited by chemical vapor deposition (CVD) onto lateral surface 18 of substrate 12 (lateral layer 20); and wire die bore 22 having wire bearing portion 24 of substantially circular cross-section and bore axis 26. Wire die bore 22 extends from top surface 14 to bottom surface 16 through substrate 12. Wire bearing portion 24 is located completely within substrate 12, and the circular cross-section of wire bearing portion 24 is determinative of the diameter of a wire drawn through the wire die bore 22. In a preferred embodiment, wire bearing portion 24 comprises a straight bore section 28 having a circular cross-section. Wire die bore 22 typically also comprises first taper 30 opening outwardly in one direction from straight bore section 28 toward top surface 14 and second taper 32 opening outwardly in the opposite direction from straight bore section 28 toward second surface 16. As illustrated in FIGS. 1-3, first taper 30 and second taper 32 are also referred to herein as entrance taper 30 and exit taper 32, respectively. A wire to be drawn initially passes through entrance taper 30 where an initial size reduction occurs prior to passing through the straight bore section 28 and exit taper 32. Referring to diamond wire dies generally, there are four main internal surfaces, commonly identified as the entrance 34, approach 36, bearing 38 and exit 40 surfaces, as shown in FIG. 1. In this description, approach 36, bearing 38 and exit 40 surfaces correspond to entrance taper 30, wire bearing portion 24 and exit taper 32, respectively. Entrance taper 30 typically extends for a greater distance along the direction of bore axis 26 than exit taper 32. Thus, straight bore portion 28 is closer to bottom surface 16 of wire die 10 than to top surface 14. There is also a wide taper 44 opening onto top surface 14 that tapers to entrance taper 28. As shown in FIG. 4, wire die 10 may also comprise top layer 46 and bottom layer 48 of diamond deposited by chemical vapor deposition (CVD) onto first surface 14 and second surface 16 of substrate 12. In such an embodiment, wire die bore 22 will extend through top layer 46 and bottom layer 48.

Typical wire drawing dies have a disc-shape, although square, hexagonal, octagonal, or other polygonal shapes may be used. The length measurement (L) as in the case of a polygonal shape, or the diameter measurement as in the case of a rounded shape, is preferably about 1-20 millimeters. Thicknesses are from 0.3-10 millimeters, with preferred thicknesses being 1-5 millimeters. The wire bearing portion 24 suitable for drawing wire is typically from 0.030 mm to 5.0 mm in diameter. Wire dies 10, as described herein, may be used to draw wire having desirable uniform properties. Wire die 10 may also contain a plurality of wire die bores 22, and these bores may have the same diameters or different diameters.

Composite diamond wire dies 10 are typically cut from a CVD coated substrate 12. Preferably, conductive CVD diamond layers can be cut by electro-discharge machining, while insulating films can be cut with a laser to form discs, squares, or other symmetrical shapes. Wire dies 10 may also be thinned to a preferred thickness, planarized or polished to a particular surface finish. These operations may be done by any suitable method, such as mechanical abrasion, laser polishing, ion thinning, or chemical methods. Prior to wire drawing, wire die 10 is mounted in a mechanical support (not shown) of a type well-known in the art in order to provide a means of holding wire die 10 during use and so as to resist axially aligned forces due to wire drawing.

Substrate 12 may be a natural diamond or a commercially available HPHT sintered diamond (e.g. Compax or Syndite available from the General Electric Company and DeBeers Company, respectively). Substrate 12 is preferably about 0.6-10 mm in width (W), which is about two times the diameter of bore 30. The width and thickness of substrate 12 should be sufficient to contain bore 26. Substrate 12 may have any suitable form, including that of a right circular cylinder or rectangular box. It is preferred that substrate 12 be free from voids and other defects that could result in pull-out in wire bearing portion 24 during wire-drawing. Also, in the case of substrates 12 formed from polycrystalline HPHT diamond, the grain boundary strength should be higher than the yield strength of the wire which is to be drawn. This is to avoid pull-out of grains or failure of the die during use. Preferably, substrate 12 comprises a single crystal of natural or HPHT diamond. It is also preferred that the <110> direction of the single crystal be oriented such that it is parallel to bore axis 26, because it is well-known that this direction offers the most desirable degree of resistance to wear and abrasion. In the case of HPHT diamond, it may be desirable to form substrate 12 from isotopically pure carbon (carbon consisting of a single isotope). Isotopically pure carbon is known to produce HPHT diamonds with enhanced thermal conductivity, on the order of 33 watts/cm<sup>2</sup>K. Since the operating temperature of wire bearing portion 24 is one of the most significant determinants of the life of a wire die, the enhanced thermal conductivity of isotopically pure substrates should translate into longer die life than would otherwise be expected for wire dies of the present invention. Substrates 12 may also be formed from macles. Macles are naturally occurring thin plates of diamond with a (111) twin plane running parallel to and midway between the main opposing surfaces of the plate. They are found in abundance in alluvial deposits. Uncoated macles have been used in the past to make wire dies, but they have only been suitable previously for drawing extremely fine wires (e.g., 0.03-0.5 mm in diameter) of relatively ductile material, because of insufficient mechanical strength resulting from their thickness (e.g., 0.1-0.5 mm). Macles are believed to offer an advantage over single crystals for use as substrate 12, because they have six <110> directions, rather than three as found in single crystals. Thus, wire bearing portion 24 formed from a macle would have six-fold rather than three-fold symmetry. Consequently, the wear of wire bearing portion 24 is expected to be more uniform, resulting in longer use of the die before repolishing of the bore.

The thickness of substrates 12 of the present invention will range from about 0.1-10 mm. Therefore, the cost of a single crystal or macle may be significantly reduced as compared to the cost of a diamond of sufficient quality and thickness necessary to form an entire wire die 10.

The combination of the thickness of lateral layer 20 should be about 0.4-10 mm, a thickness sufficient to form

the balance of the length (L) of wire die 10. A preferred technique for forming lateral layer 20 of CVD diamond is set forth in U.S. Pat. Nos. 5,110,579 and 5,387,447, respectively, which are herein incorporated by reference. According to the processes set forth in the U.S. Pat. No. 5,387,447, diamond is deposited by CVD on a substrate, which in the case of the present invention is also diamond, by a filament process. According to this process, an appropriate gas mixture containing a carbonaceous gas, such as such methane, as set forth in the example, is passed over a heated filament in a sufficient quantity, at a sufficient temperature and for a sufficient length of time to create a diamond layer and build up the layer to a desired thickness. As also described in this patent, a preferred film comprises substantially transparent columns of diamond crystals having a <110> direction perpendicular to the plane of the substrate (parallel to bore axis 26). Such a method may be used to form top layer 46 and bottom layer 48. As described in the U.S. Pat. No. 5,387,447, a uniform circumferential CVD coating may be applied to the lateral surface of a substrate. Such a method could be used to form lateral layer 20. Grain boundaries between adjacent diamond crystals having hydrogen atoms saturating dangling carbon bonds is preferred, wherein at least 50 percent of the carbon atoms are believed to be tetrahedral bonded based on Raman spectroscopy, infrared and X-ray analysis. It is also contemplated that H, F, Cl, O or other atoms may saturate the dangling carbon bonds.

The morphology of the CVD layers may also be varied using well known techniques, particularly by controlling the temperature of substrate 12 as the CVD layer is being deposited, as described for example in "Diamond Films 93", Proceedings of the 4th European conference of Diamond, Diamond-like and related Materials, Albufeira, Portugal, September 1993, Editors P. K. Bachmann, I. M. Golden, J. T. Glass and M. Kamo, Publisher: Elsevier Lausanne. Possible morphologies include: epitaxial or nearly epitaxial single crystal layers, layers comprising a plurality of large, columnar grains on the order of 50 microns or more, as well as layers that have a grain size that varies through the thickness of the layer, such as layers having a region of smaller grains near lateral surface 14 and a region of larger grains near the outer surface of wire die 10. To obtain larger grain sizes (e.g. 50 microns) or epitaxial layers, the temperature of substrate 12 during the deposition should be relatively hotter, on the order of 870°-1050° C., while smaller grain sizes (e.g. <25 microns) require temperatures on the order of 600°-850° C.

A preferred process for making the CVD layers is the filament process described herein. Additional preferred properties of these CVD diamond layers include a thermal conductivity greater than about 4 watts/cm-°K. The thermal conductivity of these CVD films may also be further enhanced by the use of isotopically pure carbonaceous gases for the CVD process, as described in U.S. Pat. No. 5,360,479 to Banholzer et al., which is herein incorporated by reference. The wear resistance and cracking resistance of wire dies 10 increases with increasing thermal conductivity. The CVD layer is preferably non-opaque or transparent or translucent and contains hydrogen and oxygen greater than about 1 part per million. The diamond film may contain impurities and intentional additives. Impurities may be in the form of catalyst materials, such as iron, nickel, or cobalt.

Diamond deposition on substrates made of Si, Ge, Nb, V, Ta, Mo, W, Ti, Zr or Hf results in CVD diamond layers that have fewer defects, such as cracks, than other substrates. By neutron activation analysis, it has been determined that

small amounts of these substrate materials are incorporated into the CVD diamond films made on these substrates. Hence, it may be desirable to adapt the processes described herein to deposit layers that contain between 10 parts per billion and less than 10 parts per million of Si, Ge, Nb, V, Ta, Mo, W, Ti, Zr or Hf. Additionally, the CVD layers may contain more than one part per million of a halogen, i.e. fluorine, chlorine, bromine, or iodine. Additional additives may include N, B, O, and P which may be present in the form of intentional additives. It is anticipated that CVD layers of the present invention may be made by other known CVD processes, such as microwave CVD processes.

It is also contemplated that CVD diamond layers having such preferred conductivity may be produced by other techniques such as microwave CVD and DC jet CVD. Intentional additives may include N, S, Ge, Al, and P, each at levels less than 100 ppm. It is contemplated that suitable films may be produced at greater levels. However, lower levels of impurities tend to increase toughness and wear resistance which are very desirable wire die properties. The most preferred films contain less than 5 parts per million and preferably less than 1 part per million impurities and intentional additives.

It is also well-known that CVD layers of the present invention may be deposited so as to contain intrinsic stresses, including intrinsic tensile stresses. For the method of deposition described herein, intrinsic tensile stresses are produced for substrate temperatures during deposition that are greater than about 740° C. The magnitude of these stresses is also known to increase with increasing temperature. Tensile stresses in the CVD layer or layers would be expected to place the substrate in compression which is known to be desirable for the purposes of decreasing the possibility of fracture within the wire die, particularly of wire bearing portion 22.

Wire die bore 26 may be formed by first piercing a pilot hole with a laser and then utilizing an ultrasonically vibrated pin in conjunction with a diamond grit slurry to abrade and form the bore by techniques known in the art.

The foregoing embodiments have been disclosed for the purpose of illustration of the present invention, and are not intended to be exhaustive of the potential variations thereof. Variations and modifications of the disclosed embodiments will be readily apparent to those skilled in the art of diamond wire dies. All such variations and modifications are intended to be encompassed by the claims set forth hereinafter.

What is claimed is:

1. A composite diamond wire die for drawing wire of a predetermined diameter, comprising:  
a substrate comprising a single crystal or a macle of natural or HPHT diamond and having a top surface, a bottom surface and a lateral surface connecting the top and bottom surfaces;  
a layer of CVD diamond containing intrinsic tensile stresses deposited on the lateral surface of said substrate (lateral layer); and  
a wire die bore comprising a wire bearing portion of substantially circular cross-section and a bore axis, said wire die bore extending from the top surface to the bottom surface through the substrate, wherein the circular cross-section of the wire bearing portion is determinative of the diameter of a wire drawn through said wire die bore.
2. The die of claim 1, wherein said substrate has a <110> direction aligned parallel to the bore axis.
3. The die of claim 2, wherein the thickness of said substrate is about 0.1-10 mm.

4. The die of claim 3, wherein the morphology of said first layer of CVD diamond comprises: 1) a region of smaller grains adjacent to said substrate and a region of larger grains adjacent to an outer surface of said first layer, 2) a plurality of large, columnar grains or 3) an epitaxial layer.

5. The die of claim 4, wherein said lateral layer has a <110> direction aligned perpendicular to the bore axis.

6. The die of claim 1, wherein said lateral layer comprises a plurality of large, columnar grains that are transparent, semi-transparent, translucent, or non-opaque.

7. The die of claim 1, wherein the top surface and the bottom surface are separated by about 0.3-10 millimeters.

8. The die of claim 1, wherein the wire bearing portion comprises a straight bore section having a circular cross-section.

9. The die of claim 8, wherein the wire die bore further comprises a first taper opening outwardly in one direction from the straight bore section toward the top surface and a second taper opening outwardly in the opposite direction from the straight bore section toward the bottom surface.

10. The die of claim 9, wherein the first taper is an entrance taper for the wire and the second taper is an exit taper.

11. The die of claim 10, wherein the entrance taper extends for a greater distance along the bore axis than the exit taper.

12. The die of claim 1, further comprising a top layer and a bottom layer of CVD diamond deposited on the top surface and the bottom surface, respectively, of the substrate, wherein a portion of said bore extends through both the top and bottom layers.

13. The die of claim 12, wherein both said top and bottom layers of CVD diamond contain intrinsic tensile stresses.

14. The die of claim 13, wherein said substrate, said top layer and said bottom layer have a thickness of about 0.3-10 millimeters.

15. The die of claim 1, wherein the wire die has outer surfaces that have been planarized or thinned by mechanical

lapping, laser polishing, or ion finishing to produce a desired surface finish or thickness of the wire die.

16. The die of claim 1, wherein said lateral layer is deposited by a process comprising passing a carbonaceous gas over a heated filament at a rate and for a time sufficient to build up the CVD layer to a desired thickness.

17. The die of claim 1, wherein said CVD diamond has a thermal conductivity greater than about 4 watts/cm-°K.

18. The die of claim 1, wherein said substrate, said lateral layer or both are formed from an isotopically pure carbonaceous material.

19. The die of claim 1, wherein said lateral layer is transparent, translucent or non-opaque and contains hydrogen and oxygen in a concentration greater than about 1 ppm.

20. The die of claim 1, wherein said lateral layer contains less than 1 ppm of impurities and intentional additives.

21. The die of claim 1, wherein said lateral layer contains more than 1 ppm of a halogen comprising fluorine, chlorine, bromine, or iodine.

22. The die of claim 1, further comprising a plurality of wire die bores each having a wire bearing portion of substantially circular cross-section and a bore axis, said wire die bores extending from the top surface to the bottom surface through the substrate, wherein the circular cross-section of the wire bearing portions are determinative of the diameter of wires drawn through said wire die bores.

23. The die of claim 1, wherein the diamond wire die is mounted in or attached to a fixture which is suitable for the support of the die.

24. The die of claim 1, wherein the diamond has an electrical resistivity of less than 1000 ohm-centimeter at room temperature.

25. The die of claim 1, wherein said lateral layer comprises a microstructure having grain boundaries, the grain boundaries comprising hydrogen saturated dangling carbon bonds.

\* \* \* \* \*